



EBERHARD HARRSCH, OF NEW YORK, N. Y.

*Letters Patent No. 90,359, dated May 25, 1869.*

**IMPROVEMENT IN THE MANUFACTURE OF COLORS.**

The Schedule referred to in these Letters Patent and making part of the same.

*To all whom it may concern:*

Be it known that I, EBERHARD HARRSCH, of New York, in the county and State of New York, have invented certain new and useful Improvements in Manufacture of Colors; and I do hereby declare that the following is a full, clear, and exact description thereof.

My invention relates to improvements in my patent, March 30, 1869, for manufacture of colors; and, to this end, consists simply in the mixing of the solutions of the ores in question, in nitric, nitro-muriatic, and muriatic acids, with salts of baryta, strontia, or their equivalents.

To enable others skilled in the art to which my invention appertains, to make and use the same, I will now describe the ingredients used.

I dissolve the ores of zinc (Franklinite, Franklinite with red oxide of zinc, amorphous zinc-ore, or the residuum, after zinc-white is driven off) in nitric, nitro-muriatic, or muriatic acids, and mix the solution with soluble salts of baryta, or carbonate of baryta, or the

same of strontia, or lime, or with the newly-precipitated oxide of zinc, or aluminium.

By precipitating any of these mixtures with ferrocyanide, bichromate, chromate, or carbonate of potassa, or soda, single or mixed, as the case may require, I gain a wider range of shades, brighter colors, and a cheaper article, than with the solutions of ores alone.

Having thus described my invention, What I claim as new, and desire to secure by Letters Patent, is—

The production of colors, by dissolving the ores of zinc in nitric, nitro-muriatic, or muriatic acids, and mixing the solution with soluble salts of baryta, or its equivalents, substantially in the manner and for the purpose described.

In testimony that I claim the foregoing as my own, I affix my signature, in presence of two witnesses.

Witnesses: **EBERH'D HARRSOH.**  
A. S. WORTH,  
JNO. A. ELLIS.